

# UNITED STATES PATENT OFFICE.

JOEL LUND, OF SAN FRANCISCO, CALIFORNIA.

## PROCESS OF SMELTING.

1,360,552.

Specification of Letters Patent. Patented Nov. 30, 1920.

No Drawing. Original application filed September 12, 1917, Serial No. 191,037. Divided and this application filed December 10, 1917. Serial No. 206,382.

To all whom it may concern:

Be it known that I, JOEL LUND, a citizen of the United States, residing at San Francisco, in the county of San Francisco and 5 State of California, have invented new and useful Improvements in Processes of Smelting, of which the following is a specification.

The object of the present invention is to provide an improved method of smelting 10 ores and metals, which will be more economical and efficient than those heretofore employed.

The present application is a division of an application filed by me September 12, 15 1917, Serial No. 191,037. In that application there was described a porous silicious substance, and a method of, and apparatus for, making the same. This substance was made by purifying molten slag, such as blast 20 furnace slag, by blowing in air and steam on the top of the slag and mixing with the molten slag granulated material of either basic or an acid nature, as required, to assist in fitting it for repeated use as a flux, 25 then causing said slag to run on to a metallic table, and puffed by fluid under pressure, then cooling the slag, then breaking it into blocks, then passing it through an alkaline 30 solution, maintaining the puffed slag as hot as possible in order that the water taken up may be evaporated therefrom as quickly as possible, leaving the solid residue in the pores of the slag, and then passing it through heated petroleum oil and coking the 35 petroleum in the pores of the slag.

It will be seen that by this process I obtain a porous, silicious material, the pores of which are filled with finely divided particles of coke obtained from the petroleum 40 oil and finely divided particles of alkaline matter precipitated from the alkaline solution. These blocks of slag, so formed, are of great value in processes of smelting ores or metal, particularly by means of fluid fuel, 45 although, as in pyrites smelting, they may be used without using fluid fuel. They may be used in blast furnaces, cupolas, and all other apparatus for smelting metalliferous material employing fluid fuel. They serve 50 to hold up the charge and render it porous; they also form a fluxing agent; the alkaline material and carbon serve as a carburizing agent; and the coke serves as a reducing agent.

55 In the smelting of the pig iron or scrap

by means of hydrocarbons or fluid fuel, it is difficult to impart to, or even to retain in, the iron a desirable amount of carbon when said iron is fused. This is caused mainly by the oxidizing action in reference to iron 60 when said fuels are used, as it has been found experimentally in the smelting of iron by the use of fluid fuel and without the addition of solid carbon that the flame exerts an oxidizing action on the metal, which result has 65 not heretofore been explained as far as I am aware. If, however, a material such as herein described, containing, or developing, a carbonate of the alkali-metals, be used to hold up the charge, said carbonates being 70 non-volatile at the high temperature necessary to carry out the process, their joint action, together with the carbon and nitrogen involved, maintains a reducing atmosphere in the zone of fusion, or, what amounts 75 to the same thing, the gases involved are maintained sufficiently carburizing in this zone, to impart to the iron the necessary carbon.

Instead of slag I may use natural pumice 80 or any porous silicious substance either natural or otherwise prepared.

I claim:—

1. In metallurgy, to flux the materials composing a charge and for other purposes, 85 the method which consists in introducing in proximity to said material in a furnace, a puffed slag in the pores of which are contained a precipitate of sodium carbonate and petroleum coke and heating said material 90 and slag.

2. In metallurgy, to flux materials composing a charge and for other purposes, the method which consists in introducing in proximity to said material in a furnace a 95 porous silicious substance, such as purified puffed blast furnace slag, in the pores of which are contained a precipitate of a carbonate of an alkali metal and coked hydrocarbon and heating said material and slag. 100

3. In metallurgy, to flux the materials composing a charge and for other purposes, the method which consists in introducing in proximity to said material in a furnace chamber such as purified puffed blast furnace slag in the pores of which are contained coked hydro-carbon and heating said material and slag. 105

JOEL LUND.